

[54] NICKEL-BASE ALLOY

[75] Inventor: Carl H. Lund, Arlington Heights, Ill.

[73] Assignee: Martin Metals Company, Wheeling, Ill.

[22] Filed: Jan. 22, 1971

[21] Appl. No.: 108,846

[52] U.S. Cl. .... 75/171

[51] Int. Cl. .... C22c 19/00

[58] Field of Search .... 75/171, 170; 148/32, 148/32.5

[56] References Cited

UNITED STATES PATENTS

3,526,499 9/1970 Quigg et al. .... 75/171

3,615,377 10/1971 Quigg et al. .... 75/171

Primary Examiner—Richard O. Dean

Attorney—John A. Crowley, Jr. and Francis J. Mulligan, Jr.

[57]

ABSTRACT

A cast nickel-base alloy containing about 5.75 percent aluminum, about 0.015 percent boron, about 0.11 percent carbon, about 10 percent cobalt, about 8 percent chromium, about 1.5 percent hafnium, about 2 percent molybdenum, about 4 percent tantalum, about 1 percent titanium, about 8 percent tungsten and about 0.08 percent zirconium.

3 Claims, 2 Drawing Figures



1000X

PATENTED AUG 21 1973

3,753,698



1000X

FIG. 1



250X

FIG. 2

CARL H. LUND

INVENTOR

BY *Carl H. Lund*  
ATTORNEY

## NICKEL-BASE ALLOY

In U.S. applications Ser. Nos. 725,074, filed Apr. 29, 1968, now abandoned and 841,505, filed July 14, 1969, now abandoned it was disclosed that addition of hafnium to certain nickel-base cast alloys resulted in various improvements in characteristics thereof. One of the alloys disclosed in that application as being improved by the addition of hafnium was identified as Alloy B. As modified with hafnium, Alloy B contained (in percent by weight) about 6 percent aluminum, about 0.015 percent boron, about 0.10 percent carbon, about 10 percent cobalt, about 8 percent chromium, about 1.5 percent hafnium, about 6 percent molybdenum, about 4.25 percent tantalum, about 1 percent titanium, about 0.075 percent zirconium with the balance being essentially nickel. Naturally, this alloy can vary in composition somewhat within a closely controlled commercial specification. As disclosed in application Ser. No. 841,505, filed July 14, 1969, now abandoned the hafnium can vary from about 1 percent to about 3 percent with the preferred amount being about 1.5 percent.

It has now been discovered that a modification of this hafnium-containing alloy wherein a major portion of the contained molybdenum is replaced by an atomic equivalent of tungsten exhibits greatly enhanced characteristics of engineering significance.

It is an object of the invention to provide a novel, highly advantageous alloy.

Another object of the invention is to provide castings made of the novel alloy of the invention having highly advantageous characteristics.

Other objects and advantages will become apparent from the following specification taken in conjunction with the drawing which illustrates the microstructure of the novel cast alloy of the present invention.

Generally speaking, the present invention comprises a cast alloy consisting, in percent by weight, of about 5.5 percent to about 6.25 percent aluminum, about 0.002 percent to about 0.05 percent boron, about the 0.07 percent to about 0.16 percent carbon, about 8 percent to about 12 percent cobalt, about 7 percent to about 9.5 percent chromium, about 0.8 percent to about 3.5 percent hafnium, about 1.5 percent to about 2.5 percent molybdenum, about 3.75 percent to about 5 percent tantalum, about 0.75 percent to about 1.5 percent titanium, about 7 percent to about 9 percent tungsten, about 0.01 percent to about 0.20 percent zirconium with the balance, except for impurities and incidental elements, being nickel. The composition of the alloy of the present invention should be balanced so as to obtain optimum cast alloy characteristics by maintaining the total of the percents of aluminum plus titanium at about 6.4 percent to about 7.2 percent and by maintaining the sum of the molybdenum percentage plus one-half the tungsten percentage at about 6 percent. As those skilled in the art will appreciate, the alloy of the present invention should be made of the purest materials commercially practical and should be melted and cast under vacuum.

An illustrative alloy of the present invention contains in percent by weight about 5.75 percent aluminum, about 0.015 percent boron, about 0.11 percent carbon, about 9.8 percent cobalt, about 7.75 percent chromium, about 1.4 percent hafnium, about 2 percent molybdenum, about 4.2 percent tantalum, about 0.9 percent titanium, about 8 percent tungsten, about 0.08

percent zirconium with the balance being essentially nickel. This alloy was melted under vacuum and cast, under vacuum using current state of the art investment casting technique, into turbine blade castings of the kind used in making turbine blades for the Pratt-Whitney JT 8D Engine. Specimens were machined from these turbine blade castings and subjected to tensile tests at room temperature and creep-rupture tests at 1,400° F. (760° C.) and at 1800° F. (872° C.). The results of these tests are set forth in the following table:

## Tensile Test (77°F.) (25°C.)

|                           |                                      |
|---------------------------|--------------------------------------|
| Ultimate tensile strength | 138.4 ksi (97.4 Kg/mm <sup>2</sup> ) |
| 0.2% yield strength       | 114.0 ksi (80.2 Kg/mm <sup>2</sup> ) |
| Elongation                | 8.6%                                 |
| Reduction in area         | 12.7%                                |

## Creep-Rupture — 1400°F. (760°C.)

|                                          |                                     |
|------------------------------------------|-------------------------------------|
| Load — 94 ksi (66.1 Kg/mm <sup>2</sup> ) | — 97 ksi (68.2 Kg/mm <sup>2</sup> ) |
| Life-to-Rupture                          | 366.6 hours                         |
| Elongation                               | 3.4%                                |
| Prior Creep                              | 3.52%                               |
| Reduction in Area                        | 10.3%                               |

## Creep-Rupture — 1800°F. (982°C.)

|                                          |
|------------------------------------------|
| Load — 29 ksi (20.9 Kg/mm <sup>2</sup> ) |
| Life-to-Rupture                          |
| Elongation                               |
| Reduction in Area                        |

The data set forth in the foregoing table shows that the alloy of the present invention exhibits, in specimens machined from cast turbine hardware, a life-to-rupture at 1,400° F. which is about four times the life-to-rupture of modified Alloy B. At 1,800° F. the life-to-rupture of the alloy of the present invention is substantially higher than the life-to-rupture of modified Alloy B.

The microstructure of the alloy of the present invention is depicted in the attached drawing under 250 X and 1000 X. The photo-micrographs were taken of alloy samples etched with an etchant made up by mixing 30 ml. of glycerol, 8 ml. of concentrated nitric acid and 6 ml. of 48 percent hydrofluoric acid.

The alloy of the present invention is particularly adapted to be used in the vacuum-cast condition as parts and structures subjected in use to high tensile forces at various temperatures extending over a temperature range of 1,000° to 1,800° F. and even higher. In particular, the alloy of the present invention is useful as parts and structures for gas turbines, said parts and structures being fabricated by investment casting technique.

While the present invention has been described in conjunction with advantageous embodiments, those skilled in the art will recognize that modifications and variations may be resorted to without departing from the spirit and scope of the invention. Such modifications and variations are considered to be within the purview and scope of the invention.

I claim:

1. A cast, nickel-base alloy consisting in percent by weight of about 5.5 percent to about 6.25 percent aluminum, about 0.002 percent to about 0.05 percent boron, about 0.07 percent to about 0.16 percent carbon, about 8 percent to about 12 percent cobalt, about 7 percent to about 9.5 percent chromium, about 0.8 percent to about 3.5 percent hafnium, about 1.5 percent to about 2.5 percent molybdenum, about 3.75 percent to about 5 percent tantalum, about 0.75 percent to about 1.5 percent titanium, about 7 percent to about 9 percent tungsten, about 0.01 percent to about 0.20 percent zirconium with the balance, except for impurities and incidental elements, being nickel.

about 1.5 percent titanium, about 7 percent to about 9 percent tungsten, about 0.01 percent to about 0.20 percent zirconium with the balance being essentially nickel, the ingredients of said alloy being interrelated such that the total of the percent aluminum plus the percent titanium is about 6.4 percent to about 7.2 percent and the total of the percent molybdenum plus 0.5 times the percent tungsten is about 6 percent.

2. An alloy as in claim 1 containing about 5.75 per-

cent aluminum, about 0.015 percent boron, about 0.11 percent carbon, about 9.8 percent cobalt, about 7.75 percent chromium, about 1.4 percent hafnium, about 2 percent molybdenum, about 4.2 percent tantalum, about 0.9 percent titanium, about 8 percent tungsten, and about 0.08 percent zirconium.

3. An alloy of claim 1 in the form of a vacuum-cast turbine blade.

\* \* \* \* \*

10

15

20

25

30

35

40

45

50

55

60

65